

## UNITED STATES PATENT OFFICE

2,552,084

WORKING FLUID FOR A COMPRESSION  
REFRIGERATION SYSTEM

Alfred E. Bishop, Oakwood, and Stanley V. Cook, Dayton, Ohio, assignors to General Motors Corporation, Dayton, Ohio, a corporation of Delaware

No Drawing. Application September 21, 1946,  
Serial No. 698,428

7 Claims. (Cl. 252—68)

1

This invention relates to chemistry and more particularly to a working fluid for use in refrigerating systems.

In refrigerating systems employing a halogenated hydrocarbon as the refrigerant, slight traces of corrosion and copper plating have been discovered. It is believed this corrosion is due to slight traces of such end products as water and hydrochloric acid probably formed by the slow break-down of the refrigerant at temperatures occurring on the high temperature side of the system. The presence of water, is also objectionable in that it may result in the formation of ice crystals on the cold or low pressure side of the system.

To overcome this latter objection it has been the custom to add to the lubricant and the refrigerant a small amount of an antifreeze such as methyl alcohol. It has been found, however, that the addition of such antifreeze increases the corrosive and copper plating action taking place within the system.

It is the object of our invention to provide a working fluid which includes in addition to the halogenated hydrocarbon refrigerant and lubricant either with or without the antifreeze, one or more organic oxides of the epoxy type acting as an inhibitor or stabilizer whereby the corrosive and copper plating actions are substantially eliminated.

As one specific example of our invention, we employ as a refrigerant difluorodichloro methane. As a lubricant, we employ mineral oil. The amount of refrigerant and the amount of the mineral oil varies with the particular refrigerating system in which the working fluid is to be used. For example, the amount of lubricant required will vary according to the amount of lubricant space provided in the compressor as well as to the efficiency of the separation of the lubricant from the refrigerant after compression and to the dependability and effectiveness of the return of the lubricant from the other parts of the system to the compressor. In general, the amount of lubricant will vary between one-fifth and an amount equal to the refrigerant by weight, depending upon the characteristics of the system wherein it is to be used. When no alcohol is to be used in the system, we include propylene oxide 1,2 in the amount of  $\frac{1}{2}\%$  to 5% of the refrigerant.

Where alcohol is to be used, we prefer to use methyl alcohol. In this event, the alcohol may be in the proportion of nine times the amount of the propylene oxide 1,2 but a greater propor-

tion of propylene oxide such as in the proportion of 2 to 3 may be used if desired. Where alcohol is used we prefer to limit the combined total of the propylene oxide and the alcohol to between  $\frac{1}{2}\%$  to 5% of the amount of the refrigerant in the system.

Instead of the particular fluorine refrigerant named above, tetrafluorodichloroethane, methyl, methylene or ethyl chloride, or one of the other refrigerants mentioned in the Midgeley et al. Resissue Patent 19,265, may be used. The mineral oil should be as free from corrosive substances as possible and of the proper viscosity characteristics. Instead of the mineral oil lubricant, other lubricants such as synthetic lubricants may be used.

Instead of the propylene oxide 1,2, the inhibitor may be selected from the other epoxy members of this same series which is termed the first ethylene oxide series. This first ethylene oxide series includes in addition to the propylene oxide 1,2, ethylene oxide, butylene oxide 1,2, butylene oxide 2,3, pentylene oxide 1,2, pentylene oxide 2,3, hexylene oxide 1,2, hexylene oxide 2,3, and hexylene oxide 3,4.

The inhibitor may also be selected from a second ethylene oxide series of epoxy type materials. This second ethylene oxide series differs from the first ethylene oxide series in that each member contains a phenyl group. This second ethylene oxide series includes phenyl ethylene oxide, phenyl propylene oxide 1,2, phenyl butylene oxide 1,2, phenyl butylene oxide 2,3, phenyl pentylene oxide 1,2, phenyl pentylene oxide 2,3, phenyl hexylene oxide 1,2, phenyl hexylene oxide 2,3, and phenyl hexylene oxide 3,4.

The members of the first and second series all include a single oxygen atom connected to two adjacent carbon atoms. Because of this structure the member of these two series are all termed epoxy type organic oxides. They have the structural formula



where R is a hydrogen atom, a methyl, ethyl, butyl, propyl, phenyl or other similar group.

These oxides may be used with various alcohols used as antifreezes in the refrigerating system, such as methyl alcohol, ethyl alcohol, normal propyl and isopropyl alcohol, normal butyl and isobutyl alcohol, tertiary butyl alcohol and benzyl alcohol. The lower alcohols appear to be more effective as antifreezes, but the higher alcohols

appear to contribute less corrosion. However, in all cases it appears that by the use of one of the members of the ethylene oxide series, particularly the propylene oxide 1,2, corrosion is effectively retarded and prevented.

While the form of embodiment of the invention as herein disclosed, constitutes a preferred form, it is to be understood that other forms might be adopted, as may come within the scope of the claims which follow.

What is claimed is as follows:

1. A working fluid for a compression refrigerating system consisting of as its major constituents a halogenated aliphatic hydrocarbon refrigerant containing not more than two carbon atoms in the molecule and a mineral oil lubricant, and as its minor constituent an organic oxide inhibitor of the epoxy type in an amount equivalent to not more than 5% of the refrigerant in the system having the following structural formula,



in which "R" and "R'" represent a hydrogen atom, a methyl, ethyl, butyl, propyl, phenyl group with the total number of carbon atoms in R and R' exclusive of the phenyl group not exceeding 4.

2. A working fluid for a compression refrigerant system consisting of as its major constituents a halogenated aliphatic hydrocarbon refrigerant containing not more than two carbon atoms in the molecule and a mineral oil lubricant, and as its minor constituents mono-hydroxy alcohol having no more than four carbon atoms in the molecule and an organic oxide inhibitor of the epoxy type having the following structural formula,



in which "R" and "R'" represent a hydrogen atom, a methyl, ethyl, butyl, propyl, phenyl group with the total number of carbon atoms in R and R' exclusive of the phenyl group not exceeding 4.

3. The method of refrigeration which consists of liquefying a halogenated refrigerant in the presence of a mineral oil and an epoxy type organic oxide inhibitor in an amount equivalent to not more than 5% of the refrigerant having the formula set forth in claim 1 hereof, and thereafter evaporating the refrigerant.

4. A working fluid for a compression refrigerating system which consists of as its major con-

stituents a refrigerant fluorochloro derivative of an aliphatic hydrocarbon having not more than two carbon atoms to the molecule and a mineral oil lubricant and has as a minor constituent phenyl ethylene oxide as an inhibitor in an amount equivalent to not more than 5% of the refrigerant.

5. A working fluid for a compression refrigerating system which consists of as its major constituents a refrigerant fluorochloro derivative of an aliphatic hydrocarbon having not more than two carbon atoms to the molecule and a mineral oil lubricant and has as a minor constituent propylene oxide 1,2, as an inhibitor in an amount equivalent to not more than 5% of the refrigerant.

6. A working fluid for a compression refrigerating system which consists of as its major constituents a refrigerant fluorochloro derivative of an aliphatic hydrocarbon having not more than two carbon atoms to the molecule and a mineral oil lubricant and has as a minor constituent phenyl ethylene oxide as an inhibitor in an amount equivalent to not more than 5% of the refrigerant and a mono-hydroxy alcohol having not more than four carbon atoms in the molecule.

7. A working fluid for a compression refrigerating system which consists of as its major constituents a refrigerant fluorochloro derivative of an aliphatic hydrocarbon having not more than two carbon atoms to the molecule and a mineral oil lubricant and has as a minor constituent propylene oxide 1,2 as an inhibitor in an amount equivalent to not more than 5% of the refrigerant and a mono-hydroxy alcohol having not more than four carbon atoms in the molecule.

ALFRED E. BISHOP.  
STANLEY V. COOK.

#### REFERENCES CITED

The following references are of record in the file of this patent:

#### UNITED STATES PATENTS

|    | Number    | Name       | Date          |
|----|-----------|------------|---------------|
| 45 | 2,040,905 | Zellhoefer | May 19, 1936  |
|    | 2,149,947 | Zellhoefer | Mar. 7, 1939  |
|    | 2,166,604 | Meyer      | July 18, 1939 |
|    | 2,185,332 | Crampton   | Jan. 2, 1940  |

#### OTHER REFERENCES

Gregory: Uses and Applications of Chemical and Related Materials, vol. II (1944). Reinhold Pub. Corp. Page 277.